

Nov. 29, 1960

E. R. HATHeway

2,962,413

METHOD OF PRODUCING CELLULOSIC PULP

Filed Oct. 19, 1956



INVENTOR.  
ERNEST R. HATHeway

BY *Hatheway & West*

ATTORNEYS

2,962,413

## METHOD OF PRODUCING CELLULOSIC PULP

Ernest R. Hatheway, 4625 Ravenwood Ave.,  
Sacramento, Calif.

Filed Oct. 19, 1956, Ser. No. 616,969

4 Claims. (Cl. 162—89)

The invention relates to improvements in the soda and the sulfate processes of making paper and other cellulosic pulps, and more particularly the production of alpha cellulose pulps in high yields and adapted for use in the chemical cellulose industry.

Historically, the soda process is one of the oldest methods of producing paper pulp. In the latter years, however, the soda process has given ground to the sulfite, or acid process; and, more recently, both the soda and sulfite processes have yielded, tonnagewise, to the sulfate process.

In all of the processes, the raw material, such as wood is appropriately prepared, as by reducing it to chips, the chips thereupon being cooked in a liquor at an elevated temperature and pressure, cooking being effected in a vessel termed a digester. Cooking is followed by washing and a series of pulp treating steps, and by bleaching.

At the conclusion of the bleaching step, the resultant pulp differs rather substantially depending on which of the processes is used. The pulp produced from both the soda and sulfite processes can generally be characterized as high white paper stock but only the stock resulting from use of the sulfite method can be further purified to yield alpha cellulose in commercial quantities. The pulp obtained from the sulfate process cannot be classified as high white paper stock; instead, the sulfate produced pulp is used in the making of heavy, strong paper such as that used in bags, cartons, etc.

Despite the numerous advantages of the soda and sulfate methods, collectively termed the alkaline processes, it has heretofore not been possible, so far as is known, to produce a high white paper stock as well as a high yield of alpha cellulose, an increasingly important and valuable raw material for the viscose and related industries, from both the soda and the sulfate processes.

Furthermore, it has heretofore been necessary, in the production of good quality paper stock and high grade alpha cellulose, to be especially selective in the wood used. Downgraded material has thus undergone a substantial reduction in value with consequent economic loss to the producer.

It is therefore an object of the invention to provide a method of producing celluloses which retains the advantages of the well-known soda and sulfate processes.

It is another object of the invention to provide a method of producing a high yield of good quality celluloses.

It is still another object of the invention to provide a method of bleaching cellulosic material to a high degree of brightness and permanence without significant loss in strength.

It is yet another object of the invention to provide a method of producing celluloses which is applicable not only to wood materials of all grades but also to wood wastes and to annual crop products, such as straw, rice hulls, bagasse, corncobs, etc.

It is another object of the invention to provide a more economical process and yet one which results in a superior product.

It is still another object of the invention to provide a method of producing a high yield of substantially pure alpha cellulose pulp and high white paper stock.

It is a further object of the invention to provide a generally improved method of producing celluloses.

Other objects, together with the foregoing, are attained in the method described in the following description and shown in the accompanying drawing in which a diagrammatic representation of the method appears.

In general, the drawing shows a conventional alkaline process flow chart; and, in the following description, the terminology employed follows the terminology long-used and wholly familiar to those skilled in the art. Consequently, unless the description calls for procedures, equipment, concentrations, reagents, temperatures, pressures, etc., differing from those presently employed in the soda and sulfate process, the traditional methods are presumed to be followed.

The process of my invention results not only in producing high white paper stock at a stage considerably in advance of that required in the present day soda process and sulfate processes, but also in producing a pulp having an alpha cellulose content in excess of 96% and an ash content of less than 0.1%, a product far superior to that realized in the conventional alkaline processes. Furthermore, by appropriate modification of some of the variables, high white paper stock and alpha cellulose yield is obtainable from annual agricultural waste plant materials such as straw, corncobs, and bagasse; and, by further modification, even rice hulls can be reduced to valuable cellulosic products, a result heretofore not achieved by any well recognized process, so far as is known, rice hulls being extremely difficult to process owing partly to their high (about 20% by weight) content of silica.

Exhaustive experiments have been undertaken to verify and establish the limits herein. California redwood (*Sequoia sempervirens*) was chosen as the subject material for the wood pulp, and rice hulls as the especial subject for agricultural plant wastes. Each is considered particularly difficult to treat, and success in their use clearly indicates, it is felt, a highly satisfactory product in the event other and more commonly used raw materials are employed.

While each of the following described departures from the conventional alkaline processes is believed to be of importance in achieving the final valuable result, it is felt that the step employed in the initial stage, wherein the material is digested or cooked in a liquor of predetermined composition, is perhaps the most important.

Whereas the "cooking liquor for the soda process consists of a solution of caustic soda containing a small amount of sodium carbonate" (Sutermeister, Chemistry of Pulp and Paper Making, Third Edition, 1941, John Wiley & Sons, New York, p. 139), the cooking liquor of the process of the invention also includes a predetermined amount of sodium, calcium, or similar hypochlorite in relation to a predetermined amount of liquor alkali as well as a predetermined liquid to solid ratio, that is to say, the ratio by weight of the cooking liquid to the dry weight of solid pulp material stock. In comparable fashion, the process of the invention also comprehends the addition of a suitable hypochlorite to the cooking or "white liquor" used in the sulfate process and which has "as its principal active constituents sodium hydroxide and sulfide" (Sutermeister, p. 107).

In the following examples, conventional sulfate liquors were used except as specific quantities of certain of the ingredients and additives are stated.

Example 1.—Redwood chips

70 Cooking liquor was prepared, the liquor in addition to other conventional sulfate liquor ingredients comprising

68 grams per liter of sodium hydroxide, 22 grams per liter sodium sulfide, 1 gram per liter sodium sulfate, and sodium hypochlorite in an amount equal to 1% of the weight of the wood chips, with a liquid to solid ratio of 5 to 1. Liquor and redwood chips were placed in a closed vessel and the temperature raised to 155° C. as rapidly as possible, approximately one hour. Temperature and vessel pressure were thereafter maintained for approximately one hour.

Digester was thereupon blown and the product subjected to the customary washing and screening operations.

Pulp was then subjected to chlorine bleaching, more than normal requirements of chlorine being used to solubalize the residual lignin and remove color. Chlorine used was equal to 5% of dry weight of wood. Chlorinated pulp was thereupon subjected to a hot sodium hydroxide extraction and then washed.

Sodium hypochlorite equivalent to 1% of the dry wood weight was then placed in solution and the pulp introduced therein to effect, after washing, a pulp of high white brightness.

At this stage the pulp constituted a high white paper stock and could be used as such. Further purification, now to be described, resulted in a high alpha cellulose pulp yield.

Purification consisted of slurry steeping (cold) in a sodium hydroxide solution of 10% NaOH for 30 minutes. The solution was thereupon recovered from the pulp by pressing, the pulp itself being subsequently shredded and then washed.

Final brightening was thereupon effected by a warm wash slightly acidified with HCl (SO<sub>2</sub> being equally satisfactory) and a subsequent filter wash. The resultant product was a high white pulp having an alpha cellulose content of 96% to 98% with an ash content less than 0.1%, the desirable and valuable properties of the cellulose having been protected, or achieved, by the relative mildness of its digestion stage in contrast to the customary alkaline process type of cooking.

Depending on the wood, variant amounts of reagents, times and temperatures are to be used. Thus, depending on the wood, the cooking liquor might contain 64 to 80 grams per liter of caustic, 1% to 2% of wood weight of hypochlorite, and a liquid-solid ratio of 5 to 1 to 6 to 1. Temperature of cooking can range from 155° C. to 165° C. depending on the wood, with time in coming up to temperature varying from one hour to one hour and a quarter, and time of holding at temperature and vessel pressure ranging from one to one and one-half hours. In the chlorination bleaching step, the amount of chlorine used may vary from 5% to 8% of the wood weight, again depending on the type of wood treated. The sodium hydroxide, furthermore, used in the purification process can vary from 10% to 12.5%, with the slurry steeping period ranging from 30 minutes to one hour.

The use of hypochlorite in the cooking liquor represents a radical departure from classical alkaline process practice, the hypochlorite permitting the use of the less expensive alkaline processes in the production at an early stage of high white paper stock and the efficient production of high grade alpha cellulose pulp, a result heretofore considered unattainable economically in commercial yields.

The first reaction of hypochlorite in a highly alkaline cooking liquor is chlorination. This moderate chlorination at an early stage in the treatment results in a more easily bleachable pulp. The amount of hypochlorite used, as well as the time and temperature of the cook, must be controlled so that the maximum amount of available chlorine in the hypochlorite is directed to chlorination and as little as possible to oxidation. This situation is critical since hypochlorite under certain conditions has a high oxidation potential. Increasing the temperature above the maximums herein described results in marked

degradation of the cellulose. The use of hypochlorite in the cooking stage, in addition to its other valuable contributions, permits of some degree of viscosity control, a factor of especial importance to the viscose and chemical cellulose industry.

5 While the process can be applied to all woods and wood wastes, including redwood and redwood bark, it has been found that, owing to the unusual properties of redwood bark, digestion is preferably carried on without vessel pressure and at a temperature of 95° C. to 100° C.

10 In somewhat comparable fashion, in the case of all annual plant waste materials, with the exception of rice hulls, digestion is preferably carried on at atmospheric pressure, within a temperature range of 95° C. to 100° C. and at a liquid solid ratio of 10 to 1.

*Example 2.—Rice hulls*

Digestion was carried out using a cooking liquor comprising, among other conventional sulfate liquor ingredients, 80 grams per liter of NaOH, sodium hypochlorite equal to 2% of hull weight, with a liquid-solid ratio of 10 to 1. Time of coming up to 140° C. temperature in closed vessel was one hour, with pressure being maintained for one hour and a half.

25 The charge was then blown and the pulp washed and screened, with rejects going to a suitable refiner for later return.

30 Chlorine was thereupon introduced into the pulp under agitation for 30 minutes at a rate of 0.25% of the weight of the hulls per minute. Chlorine flow was then shut off and agitation of the pulp continued for 20 to 30 minutes to consume all free chlorine in the liquid medium.

35 After washing, the pulp was subjected to a hot sodium hydroxide extraction for a period of one hour at which point the pulp was again washed.

40 A single stage hypochlorite bleach was then effected, using the hypochlorite equivalent of 1% of the weight of the hulls. This step was carried out at a temperature not in excess of 50° C. for a period of one hour, washing then being performed.

The charge at this juncture constituted high white pulp.

Purification was thereupon undertaken, comprising cold steeping for one hour using a 10% to 12.5% sodium hydroxide solution, followed by pressing, with the recovered solution being directed to storage for cooking liquor make-up, then by pulp shredding and washing.

45 The final brightening wash was thereupon made in hot water slightly acidified, followed by a clear wash.

50 The pulp at this point was of high white brightness and had an alpha cellulose content in excess of 96% and ash content of less than 0.1%.

55 As can be seen, even redwood and rice hulls, when processed by the improved alkaline methods of the invention, provide without the return cycling steps ordinarily required, either a high white paper stock or, in the event purification is undertaken, a high yield of high quality alpha cellulose. It is again emphasized that the improved process can be used with conventional cooking liquors of the soda or sulfate processes, with the departures described, and that the process of the invention is wholly compatible with the equipment presently used in the two alkaline processes.

60 What is claimed is:

1. An improved process of producing high white paper stock from wood comprising the steps of adding to an alkaline process cooking liquor having a sodium hydroxide concentration of 64 to 80 grams per liter and a liquid to solid ratio of 5 to 1 to 6 to 1 a hypochlorous acid salt 1% to 2% by weight of the weight of the wood.
- 65 70 of bringing the temperature of the cooking liquor to 155° C. to 165° C. within one hour to one hour and a quarter, of maintaining said temperature for a period of one hour to one hour and a half, of blowing the digester, of screening the pulp, of subjecting the pulp to a chlorination bleach, of washing the pulp, of subjecting the pulp

to a hot sodium hydroxide extraction, of washing the pulp, of bleaching the pulp in a solution of sodium hypochlorite equivalent to 1% of the weight of the wood, and of washing the pulp.

2. The steps of claim 1 followed by purification comprising the steps of steeping the pulp in a cold solution of 10% to 12.5% sodium hydroxide from one half hour to one hour, of pressing said sodium hydroxide solution from the pulp, of shredding the pulp, of washing the pulp and of brightening the pulp in a slightly acidified warm wash, and of washing the pulp to yield a purified high white pulp having an alpha cellulose content in excess of 96% by weight and with an ash content of less than 0.1% by weight.

3. An improved alkaline process of producing valuable 15 cellulosic products from rice hulls comprising the steps of digesting the hulls in a cooking liquor having a sodium hydroxide concentration of 80 grams per liter and a hypochlorite concentration of 2% by weight of the weight of the rice hulls, said digesting step including bringing the 20 charge up to a temperature of 140° C. in a closed vessel in one hour and of maintaining said temperature for one hour and a half, of blowing, washing and screening the charge, of subjecting the charge to a first chlorination including introducing chlorine into the charge under agitation for 30 minutes at a rate of 0.25% of the rice hull weight per minute, of agitating the pulp for 20 to 30 25

minutes thereafter, of subjecting the pulp to a hot sodium hydroxide extraction for one hour, of washing the pulp, of bleaching the pulp using a solution of hypochlorite equivalent to 1% of the weight of the rice hulls, at a temperature not in excess of 50° C. for one hour, and of washing the pulp.

4. The steps of claim 3 further characterized by a purification operation including cold steeping the pulp for one hour in a 10% to 12.5% sodium hydroxide solution, of pressing, shredding and washing the pulp, and of brightening the pulp in slightly acid hot water bath.

References Cited in the file of this patent

UNITED STATES PATENTS

|           |                  |               |
|-----------|------------------|---------------|
| 1,196,708 | McCormack et al. | Aug. 29, 1916 |
| 1,235,258 | Toles            | July 31, 1917 |
| 1,557,338 | Runkel           | Oct. 13, 1925 |
| 1,570,389 | Morgenier        | Jan. 19, 1926 |
| 1,773,320 | Richter          | Aug. 19, 1930 |
| 1,858,523 | Richter et al.   | May 17, 1932  |
| 1,859,224 | Swan             | May 17, 1932  |
| 2,249,174 | Richter          | July 15, 1941 |
| 2,698,233 | Lewis et al.     | Dec. 28, 1954 |

FOREIGN PATENTS

|         |               |               |
|---------|---------------|---------------|
| 298,333 | Great Britain | Oct. 11, 1928 |
| 471,695 | Canada        | Feb. 20, 1951 |